

## UNITED STATES PATENT OFFICE

2,406,337

## MODIFICATION OF FATTY OILS

Laszlo Auer, South Orange, N. J.

No Drawing. Application January 23, 1943,  
Serial No. 473,396

22 Claims. (Cl. 260—407)

1

## GENERAL FIELD OF INVENTION AND STATEMENT OF OBJECTS

This invention relates to the modification of fatty oils, and especially to drying and semi-drying fatty oils.

Fatty oils are employed in a number of different industries, such, for instance, as the coatings and plastics industries, and it is a general object of this invention to modify and improve the properties of fatty oils for various industrial purposes.

Briefly, the invention contemplates treatment of a fatty oil, for instance, linseed oil, with polyhydroxy benzenes, such as dihydroxy and trihydroxy benzenes, the mixture being heated to elevated temperatures. I have secured particularly good results with resorcinol, which is a dihydroxy benzene. Full description of the treatment procedure is given hereinafter.

According to the present invention, it is possible to achieve a number of advantages in the treatment of fatty oils. For example, it is possible to materially improve the drying characteristics of the fatty oil, and also to improve water and alkali resistance of film coatings or the like formed with the treated oil.

The foregoing and other objects and advantages will appear more fully hereinafter, especially from consideration of examples given. Before proceeding with description of the treatment procedure, reference is now made to the fatty oil materials to which the invention is applicable.

The process may be employed on fatty oils generally, including drying oils, semi-drying oils, and non-drying oils. The following is a typical list of such oils:

- Tung oil
- Oiticica oil
- Dehydrated castor oil
- Linseed oil
- Perilla oil
- Sunflower oil
- Poppyseed oil
- Soya bean oil
- Walnut oil
- Rapeseed oil
- Pine seed oil
- Olive oil
- Corn oil
- Cottonseed oil
- Coconut oil
- Babassu oil
- Hydroxylated oils such as castor oil, etc.
- Fish oils (train oils)

2

In addition, it should be noted that esters of fatty acids other than the natural glycerin esters (fatty oils) may be used, for example, synthetic glycerin esters of fatty acids, and fatty acid esters formed with other polyhydric alcohols, such as glycols, pentaerythritol, mannitol, sorbitol, etc. For convenience, all such materials are herein referred to merely as fatty oils.

The process may be employed on fatty oils themselves or on various mixtures of materials containing fatty oils, for instance, on varnishes or varnish bases of oleo-resinous types, whether used clear or pigmented. Reference herein to "varnish base" means all or part of the varnish solids or film forming ingredients.

Fatty acids may be added to the reaction mixture, if desired.

## TREATMENT PROCEDURE AND CONDITIONS

20 As above noted, the treatment process involves heating the fatty oil, or the material containing same, in the presence of a polyhydroxy benzene, especially dihydroxy and trihydroxy benzenes. Particularly good results have been secured by the 25 use of resorcinol which is a dihydroxy benzene; and with pyrogallol, which is 1, 2, 3 trihydroxy benzene.

The quantity of treating agent employed may be varied over a considerable range, depending 30 upon the extent of modification desired, the temperature, the particular fatty oil being treated, etc. From a small fractional percentage, for instance, from about 0.05% or 0.1% up to about 35% may be used, although ordinarily from about 0.5% to about 5 or 10%, for instance, 2% is quite effective.

In connection with treatment temperature, it may be said that in general temperatures from about the lowest dissolution temperature of the 40 modifying agent up to about 350° C. are usable, although the temperature should not be above the point at which the fatty oil appreciably decomposes.

The time of treatment will vary in accordance 45 with other factors such as temperature, percentage of treating agent, etc. Ordinarily the time should be at least 30 minutes and most usually several hours, for instance, from about 1 hour to about 5 hours.

50 In connection with treatment procedure, it is pointed out that the treatment of a fatty oil may be effected by adding the treating agent and heating the oil under conditions mentioned above. If desired, the treating agent may also be mixed 55 with a varnish base or other composite material

incorporating a fatty oil material, such composite material then being heated under conditions such as those discussed above.

Agitation may advantageously be used during any mixing procedure, in order to aid thorough dispersion of the treating agent.

The treatment may be carried out under varying atmospheric conditions, both with respect to pressure and also with respect to the gas in contact with the reaction mixture. Thus, under some circumstances, the fatty oil or the mixture containing the fatty oil may be heated under vacuum, and under other conditions, atmospheric pressure may be used, and also superatmospheric pressure.

It is frequently of advantage to exclude the air from the reaction mixture and this may be done during any stage of treatment, either by employing vacuum or by blanketing the surface of the batch with some non-oxidizing or inert gas, for instance,  $\text{CO}_2$ ,  $\text{SO}_2$ ,  $\text{H}_2\text{S}$ , or nitrogen. Still further, exclusion of air may be obtained by carrying out the reaction in a closed vessel (but not necessarily under a positive pressure), in which event vapors or the like released from the reaction mass may serve to dispel or exclude the air. I have found vacuum treatment to be particularly effective, for instance, from about 100 mms. Hg to about 450 mms. Hg internal pressure, although higher or lower pressures are also useable.

With regard to the foregoing atmospheric conditions in the reaction vessel, it may be noted that certain of the gases mentioned may be employed for their supplemental effect on the reaction, in which event, if desired, the gases may be bubbled through the reaction mixture.

In general, it may be pointed out that increasing any one of the variables: temperature, time or percentage of modifying agent, usually increases the rate and/or extent of the reaction.

The modifying agents herein claimed may be employed (either simultaneously or sequentially) in combination with others disclosed, for instance, in various of my copending applications and issued patents, some of which are mentioned hereinafter.

In addition, supplemental treatments may be applied to the oil, either during or following the reaction with the agents here contemplated, many of such supplemental treatments also being discussed fully in copending applications and issued patents below mentioned. For instance, the modified oil products may be vulcanized with sulphur or sulphur chloride or similar vulcanizing agents.

Attention is directed to my copending application Serial No. 461,789, filed October 12, 1942, which discloses treatment of fatty oils with fluorescein and also with a combination of phthalic anhydride and resorcinol.

Where a fatty oil is being treated to prepare it for incorporation in a varnish base of the oleoresinous type, one particularly advantageous procedure is as follows: In this case the treating agent may initially be added to and dispersed in the fatty oil at relatively low temperature, for instance, from about 75° C. to about 200° C.; and then when the oil is incorporated in the varnish or varnish base, additional heating may be applied at higher temperatures, in order to carry out the full degree of modification of the oil contemplated.

Even when treating a fatty oil alone, it may be advantageous to divide the treatment into two stages, the first of which is carried on at a relatively low temperature, and the latter of which is carried on at a higher temperature.

Wherever the two-stage type of procedure is adopted, it may be advantageous to carry on the first stage, at relatively low temperature, under pre-condensation conditions, especially when employing certain of the treating agents contemplated, such as resorcinol which displays a marked tendency to sublime. A reflux condenser will be found effective in reducing the effect of sublimation.

By proceeding in this way (pre-condensation at relatively low temperature followed by additional heating at a higher temperature), loss of treating agent is prevented or at least reduced.

The term "pre-condensation" (initial or primary condensation), as used herein, means treatment under conditions of the type just mentioned at temperatures below the sublimation point and for a time such that upon subsequent heating of the treated oil to higher or heat bodying temperatures the resorcinol no longer tends to sublime to any great extent.

#### EXAMPLES

In order to demonstrate the process linseed oil and resorcinol were selected as typical of the starting materials and treating agents, these two being used in most of the examples given below.

To determine the most advantageous treatment conditions, several comparative series of experiments were carried out, all utilizing resorcinol and linseed oil. An analysis of these experiments will aid in an understanding of the invention.

First, note that resorcinol has a boiling point of 276.5° C., and melts at 116° C. When molten, it dissolves quite easily in fatty oils and even at temperatures below its melting point, it is soluble in many fatty oils.

In spite of the fact that the boiling point of resorcinol is comparatively high, it sublimes out of fatty oils at temperatures below its boiling point. Furthermore, its boiling point is below the usual and preferred temperature range for bodying fatty oils or for cooking varnishes.

#### COMPARATIVE EXAMPLES 1 TO 5

Because of the foregoing characteristics, it is advantageous to adopt some means or procedure for reducing loss of the treating agent by sublimation or boiling. With this in mind, a series of experiments were carried out in one liter aluminum beakers provided with covers, using resorcinol and alkali refined linseed oil, in 400 gm. batches, each being heated at a different temperature, as is indicated in Table No. I—A, herebelow, showing reaction conditions and the resulting viscosities of the treated oils. All viscosities given herein are expressed in terms of the Gardner Holt scale.

In all cases of this series 2% of resorcinol was used and the temperature was maintained for 2 hours.

Table No. I—A  
ALKALI REFINED LINSEED OIL WITH RESORCINOL  
IN COVERED KETTLE

| Ex. No. | Temperature                     | Viscosity | Extent of sublimation |
|---------|---------------------------------|-----------|-----------------------|
| 1       | 100° C.                         | A         | Slight.               |
| 2       | 150° C.                         | A         | Considerable.         |
| 3       | 200° C.                         | B+        | Do.                   |
| 4       | 250° C.                         | B+        | Do.                   |
| 5       | 300° C.                         | S         | Do.                   |
| A       | (The same oil without heating.) | A         |                       |

The foregoing series indicated that sublima-

tion increased in general with increase in temperature.

Following the initial treatment of the several batches as mentioned above, varnishes were prepared with the treated oils, the several varnishes then being subjected to drying and water tests with results indicated in Table No. I-B herebelow. The varnishes were prepared with ester gum, each being of 25 gallon length, and each varnish was cooked at 300° C. to a viscosity of about C to D, at 50% solids when thinned with mineral spirits. The cooking time required to reach this viscosity is indicated in the table below.

An explanation of the designations under the drying and other test columns is given after the table, but it is here pointed out that the following as well as other tables, appearing in the present specification, include (in addition to numbered examples) lettered examples which represent "blank" or "control" experiments, i. e., an experiment carried out with the same oil, under exactly the same treatment conditions as the numbered examples, except that no treating agent was used. It may also be mentioned that statements regarding comparisons of properties, such as drying characteristics, are always related to films formed with varnishes incorporating the same fatty oil treated under the same conditions (both prior to and during the formation of the varnish itself) but without the presence of the modifying or treating agent.

In the table just below the example numbers correspond to those in Table No. I-A, the letter "v" following the example number indicating the 35 varnish prepared with the treated oil.

The cold water test was carried out by immersing one half of each panel (carrying the varnish film) in cold water for 24 hours; and observing the milkiness of the film and the rate of recovery to the original condition. The hot water test was carried out in a similar manner, except that the panels were immersed in boiling water for 15 minutes; the milkiness and rate of recovery again being observed.

10 The columns under the "Cold water" and "Hot water" headings indicate the following:

Con=arbitrary scale of condition of film when first removed after the test, No. 1 indicating the best condition.

15 Rec=arbitrary scale representing rate of recovery to original condition after withdrawing from the test, No. 1 indicating the best rate.

ON=arbitrary scale of the condition of the film after standing overnight (following immersion period), No. 1 indicating the best condition.

20 The alkali resistance test was carried out with somewhat heavier films than for the drying test, and cold water and hot water tests. For this purpose films of 0.003" thickness were applied to test panels which were then immersed in a 3% aqueous sodium hydroxide solution. The condition after 7 hours immersion was observed and recorded, and also the condition after overnight immersion. 25 The results of these two observations are indicated in the corresponding columns under the heading "Alkali." The key to the letters in these columns is as follows:

H=hazy

Sl.m=slightly milky

M=milky

Table No. I-B

VARNISHES PREPARED WITH TREATED OILS OF TABLE NO. I-A

| Ex. No. | Minutes cooking at 300° C. | Viscosity | Drying |     |     |    | Cold water |     |     | Hot water |     |     | Alkali |        |       |
|---------|----------------------------|-----------|--------|-----|-----|----|------------|-----|-----|-----------|-----|-----|--------|--------|-------|
|         |                            |           | Set    | DF  | TF  | ON | 48         | Con | Rec | ON        | Con | Rec | ON     | 7 hrs. | ON    |
| 1v      | 164                        | A         | 1/2    | 3/4 | 1   | B  | A          | 3   | 2   | 2         | 5   | 2   | 2      | Sl. m. | M-40. |
| 2v      | 207                        | C         | 1/2    | 1/2 | 1   | D  | A          | 2   | 1   | 1         | 5   | 2   | 1      | M      | M-20. |
| 3v      | 203                        | C         | 1/2    | 3/4 | 3/4 | B  | A          | 2   | 1   | 1         | 5   | 1   | 1      | Sl. m. | M-40. |
| 4v      | 185                        | C         | 1/2    | 3/4 | 3/4 | C  | B          | 4   | 2   | 1         | 6   | 2   | 1      | M      | M-20. |
| 5v      | 161                        | D         | 1/2    | 3/4 | 3/4 | C  | A          | 2   | 1   | 1         | 5   | 1   | 1      | M      | M-30. |
| Av      | 190                        | C         | 1      | 2   | 2   | D- | A          | 1   | 1   | 1         | 5   | 3   | 2      | M-80.  | Gone. |

All varnish tests in the present series, as well as in other series of examples mentioned herein-after, were carried out in the following manner. Initially the varnishes were stored for 48 hours after the addition of driers (0.3% lead, 0.03% cobalt and 0.02% manganese, based on the oil content of the varnish and added in the form of naphthenate driers). In order to test the characteristics of the varnishes, a coating knife yielding a film of 0.0015" thickness was employed.

The columns under the heading "Drying" indicate the following:

Set=time in hours to initially set.

DF=time in hours for the film to become dust-free.

TF=time in hours for the film to become tack-free.

ON=condition of film after "overnight" drying, the letters representing an arbitrary scale to indicate the relationship between the several examples, and also their relation to the item just below (the letter A indicates the driest film and succeeding letters progressively decrease in hardness).

48=condition of film after drying for 48 hours.

55 Where appreciable dissolution of the film took place, that fact is noted in the corresponding columns by figures, representing the approximate percentage of the film remaining. For instance, M-40 indicates that the film was milky and that 40% of the immersed part of the film remained on the panel, 60% being destroyed.

60 With the foregoing explanatory comments in mind, it will be seen from Table No. I-B that notwithstanding the appreciable loss in treating agent during the initial treatment of the oil (see Table I-A), the varnish films displayed considerable improvement in a number of respects as compared with a film made from a varnish incorporating the same oil in untreated condition (compare Example Av with the others). The alkali resistance and drying characteristics both display considerable improvement.

COMPARATIVE EXAMPLES 6 TO 9

70 In this series of examples alkali refined linseed oil was also used and was treated with 2% resorcinol, as in the first series. In each case a batch of 400 gms. of oil was placed in a one liter Erlenmeyer flask equipped with a reflux condenser, so as to provide a condition of pre-con-

densation and thereby reduce loss of the resorcinol. For the reflux condenser, a straight air condenser was used, since the relatively high boiling point of resorcinol does not necessitate water cooling. In all experiments of this series the refluxing time was two hours. The temperatures tried differed as between different examples, the results being indicated in the Table II—A herebelow.

Table No. II—A

## ALKALI REFINED LINSEED OIL WITH RESORCINOL UNDER REFLUX

| Ex. No. | Temperature                                      | Viscosity | Extent of sublimation |
|---------|--------------------------------------------------|-----------|-----------------------|
| 6       | 150° C.                                          | A         | Very little.          |
| 7       | 200° C.                                          | B         | Do.                   |
| 8       | 250° C.                                          | C         | Do.                   |
| 9       | 300° C.                                          | T         | Do.                   |
| B       | (The same oil without heating and not refluxed.) | A         |                       |

As in Examples 1 to 5, the treated oils of Examples 6 to 9 were also used in preparing ester gum varnishes of 25 gallon length, the formulation being the same as described above. These varnishes were then tested and the results are indicated in Table II—B just below, incorporating columns and distinctions corresponding to those described above.

Table No. II—B  
VARNISHES PREPARED WITH TREATED OILS OF TABLE NO. II—A

| Ex. No. | Minutes cooking at 300° C. | Viscosity | Drying |     |     |     | Cold water |     |     | Hot water |     |     | Alkali |        |       |
|---------|----------------------------|-----------|--------|-----|-----|-----|------------|-----|-----|-----------|-----|-----|--------|--------|-------|
|         |                            |           | Set    | DF  | TF  | ON  | 48         | Con | Rec | ON        | Con | Rec | ON     | 7 hrs. | ON    |
| 6v      | 189                        | C         |        | 1/2 | 1/2 | 3/4 | B          | A   | 3   | 1         | 1   | 5   | 1      | 1      | H.    |
| 7v      | 210                        | D         |        | 1/2 | 1/2 | 1   | C          | A   | 2   | 2         | 2   | 5   | 2      | 1      | M-80. |
| 8v      | 210                        | D         |        | 1/2 | 1/2 | 3/4 | B          | A   | 2   | 1         | 1   | 6   | 1      | 1      | H.    |
| 9v      | 105                        | D         |        | 1/2 | 1/2 | 3/4 | D          | A   | 1   | 1         | 1   | 5   | 1      | 1      | H.    |
| Bv      | 190                        | C         | 1      | 2   | 2   | D-  | A          | 1   | 1   | 1         | 5   | 3   | 2      | M-80.  | Do.   |

The faster bodying of the varnish of Example 9v may be partly explained by the fact that the oil here employed (see Table II—A) had a much higher viscosity than the other oils, indicating that at least a portion of the bodying took place during refluxing.

The foregoing table shows that cold and boiling water resistance and also the alkali resistance were quite satisfactory and further that

## COMPARATIVE EXAMPLES 10 TO 12

In a third comparative series of examples, alkali refined linseed oil was again used and the percentage of resorcinol was varied in order to indicate what percentages yielded the best results.

In the examples of this series 4,000 gm. batches of the oil were placed in stainless steel kettles of three gallon size, the kettles being covered and provided with an air condenser. In each case a blanket of CO<sub>2</sub> was maintained at the surface of the oil and all of the oils were heated under reflux preliminarily for two hours at 200° C. and thereafter for an additional period at 300° C. for a time sufficient to increase the body to from about Z4 to Z6 viscosity. Results of this series of examples are indicated in Table No. III—A.

Table No. III—A  
ALKALI REFINED LINSEED OIL WITH VARYING PERCENTAGE OF RESORCINOL

| Ex. No. | Percentage | Time at 300° C.  | Viscosity |
|---------|------------|------------------|-----------|
| 10      | 0.5%       | 8 hrs., 10 mins. | Z5        |
| 11      | 2.0%       | 8 hrs., 40 mins. | Z4        |
| 12      | 4.0%       | 7 hrs.           | Z6        |
| C       | No agent   | 8 hrs., 20 mins. | Z5        |

From the above it will be seen that lower than

about 4% of resorcinol does not materially accelerate the rate of bodying.

To demonstrate drying and other characteristics of these treated oils, 25 gallon length ester gum varnishes were again prepared and cooked in a manner similar to those described above, except that the viscosity attained was about from C to E. The properties of these varnishes are indicated in Table III—B just below.

Table No. III—B  
VARNISHES PREPARED WITH TREATED OILS OF TABLE NO. III—A

| Ex. No. | Minutes cooking at 300° C. | Viscosity | Drying |       |    |    | Cold water |     |     | Hot water |     |     | Alkali |        |       |
|---------|----------------------------|-----------|--------|-------|----|----|------------|-----|-----|-----------|-----|-----|--------|--------|-------|
|         |                            |           | Set    | DF    | TF | ON | 48         | Con | Rec | ON        | Con | Rec | ON     | 7 hrs. | ON    |
| 10v     | 95                         | C         | 1 1/2  | 3     | 4  | B  | A          | 2   | 2   | 1         | 6   | 5   | 5      | M.     | Gone. |
| 11v     | 116                        | C         | 1 1/2  | 2     | 3  | B  | A          | 2   | 2   | 1         | 5   | 2   | 2      | Sl. m. | Do.   |
| 12v     | 90                         | D         | 1 1/2  | 3     | 3  | D  | A          | 1   | 1   | 1         | 6   | 5   | 5      | H.     | Do.   |
| Cv      | 135                        | E         | 1/2    | 1 1/2 | 2  | D- | A          | 2   | 2   | 1         | 5   | 1   | 1      | H.     | Do.   |

the drying of the varnishes made with treated oils was distinctly improved. The drying of the varnishes made with oil refluxed at 150° C. (varnish 6v) and at 250° C. (varnish 8v) was the best, the former having a slight edge over the latter. The drying of the varnishes containing the treated oils was in all cases extensively improved as compared with the blank experiment (Bv).

From the above it appears that pre-condensation by refluxing between about 150° C. and 250° C. gives the most advantageous results.

From the foregoing, it may be noted that while the resorcinol, when used in low percentages, does not appear to appreciably accelerate the rate of bodying of the oils, nevertheless, considerable improvement with respect to rate of bodying is observable in preparing or cooking the varnishes from the pre-treated oils.

The varnishes made with oil containing 0.5% resorcinol (10v) and 2% resorcinol (11v) both showed up quite well in various of the drying and other tests. The varnish containing 2% resorcinol (11v) seems to yield the best results.

## EXAMPLE 13

Further tests were made employing different percentages of resorcinol with linseed oil, the different percentages having been obtained by diluting a precondensed concentrate with additional oil. These tests were carried out in the following manner:

Initially a batch of alkali refined linseed oil was treated with 2% of resorcinol under precondensation conditions at a temperature of 150° C. for 2 hours. This treated batch was then diluted with additional alkali refined linseed oil in order to secure test batches incorporating the following percentages of resorcinol.

| Example No. | Resorcinol |
|-------------|------------|
| Per cent    |            |
| 13a         | 1.0        |
| 13b         | 0.5        |
| 13c         | 0.2        |
| 13d         | 0.1        |
| 13e         | 0.05       |

Heavy bodied oils were prepared of each of the diluted oils, and also of a portion of the 2% batch initially prepared, by bodying them to Z-4 to Z-6 viscosity.

Varnishes were then prepared with each of the above heavy bodied oils. These varnishes were prepared with ester gum in twenty-five gallon length, and each varnish was cooked to a standard viscosity.

All of the varnishes were tested in accordance with the methods set out above, and in general all batches showed improvements in at least certain respects, as compared with a similar varnish made in essentially the same way but not containing resorcinol-treated oil. Some of the specific results were as follows:

In cold water resistance, the 2% resorcinol containing oil yielded the best results, although these results were approached by the varnish prepared with the 0.05% resorcinol containing oil. In the boiling water test, the results were similar to those in cold water.

In alkali resistance, the several batches may

ing the oil under pre-condensation or refluxing at a temperature of about 150° C. and for a time of about two hours. That these conditions constitute about the most favorable balance, when considering the various different characteristics and properties, is further evidenced by the results of another comparative series of examples given just below.

## COMPARATIVE EXAMPLES 14 TO 17

In this series of examples alkali refined linseed oil was again used and in each example 2% of resorcinol was employed as the treating agent. The batch of each example was preliminarily heated under reflux for two hours, the refluxing temperature being different as between the several examples. Thereafter, the treated oil of each batch was heat bodied at 300° C. for a time of about 3 1/4 hours. The viscosities obtained in the given time are indicated in Table IV-A just below.

Table No. IV-A

## HEAT BODYING OF RESORCINOL TREATED ALKALI REFINED LINSEED OIL

| Ex. No. | Reflux temperature | Time at 300° C. to heat body | Viscosity |
|---------|--------------------|------------------------------|-----------|
| 14      | 150                | 3 hrs., 20 min.              | Z-5       |
| 15      | 200                | 3 hrs., 15 min.              | Z         |
| 16      | 250                | 3 hrs., 20 min.              | Z-2       |
| 17      | 300                | do                           | Z-6       |

The foregoing indicates that refluxing at about 150° C. results in quite rapid bodying during the subsequent heat bodying. The relatively high viscosity (Z-6) secured with the oil refluxed at 300° C. (Example 17) is apparently due to the fact that at least a portion of the heat bodying took place during the refluxing itself.

Ester gum varnishes of twenty-five gallon length were prepared from the foregoing bodied oils, the preparation being according to the formula and process already described above in connection with other examples. The drying and other properties of the varnishes thus prepared are indicated in the following table.

Table No. IV-B

| Ex. No. | Minutes cooking at 300° C. | Viscosity | Drying |     |    |    | Cold water |     |     | Hot water |     |     | Alkali |        |       |
|---------|----------------------------|-----------|--------|-----|----|----|------------|-----|-----|-----------|-----|-----|--------|--------|-------|
|         |                            |           | Set    | DF  | TF | ON | 48         | Con | Rec | ON        | Con | Rec | ON     | 7 hrs. | ON    |
|         |                            |           |        |     |    |    |            |     |     |           |     |     |        |        |       |
| 14v     | 60                         | C         | 1/2    | 3/4 | 1  | B  | A          | 1   | 1   | 1         | 5   | 1   | 1      | H      | M.    |
| 15v     | 90                         | D         | 2/2    | 2/4 | 1  | D  | A          | 1   | 2   | 1         | 5   | 1   | 1      | H      | M-70. |
| 16v     | 90                         | D         | 2/2    | 2/4 | 1  | C  | A          | 2   | 1   | 1         | 5   | 1   | 1      | SI. m. | Gone. |
| 17v     | 55                         | O         | 1/2    | 3/4 | 1  | B  | A          | 2   | 1   | 1         | 6   | 1   | 1      | M.     | M-20. |

be graded in the following order of percentage of resorcinol contained in the oil used, the first figure showing the best results and the others gradually decreasing in alkali resistance: 1%, 0.5%, 0.05%, 0.2%, 2%, and 0.1%.

From this series of tests it will be seen that certain of the properties of the treated oils and varnishes made therefrom are not necessarily proportional to the quantity of resorcinol present. Therefore, for individual uses and applications, the concentration most favorable to that purpose should be selected.

Various of the foregoing comparative examples indicate that for an all round type of product, an effective balance of desirable properties is secured by the employment of resorcinol in an amount approximating 2% and by pretreat-

ing the oil under pre-condensation or refluxing at a temperature of about 150° C. and for a time of about two hours. That these conditions constitute about the most favorable balance, when considering the various different characteristics and properties, is further evidenced by the results of another comparative series of examples given just below.

As hereinbefore mentioned, for certain purposes it may be desirable to treat the oil not only with resorcinol or other polyhydroxy benzenes, but also with some other agent or agents. This may be advantageous where it is desired to improve certain specific properties, for instance, alkali resistance, drying, speed of varnish bodying, etc. Examples of such composite treatment are given below.

## EXAMPLE 18

A batch of 4,000 gms. of alkali refined linseed oil was heated with 0.5% sulpho-salicylic acid at 100° C., until the reagent dissolved. The heating was carried out in a three gallon open kettle with a blanket of CO<sub>2</sub>. After dissolution of the sulpho-salicylic acid, 2% of resorcinol was added to the oil and a cover applied, with a reflux condenser on the kettle. The oil was then heated at 150° C. for two hours, to effect pre-condensation.

For purposes of comparison two additional batches of oil were prepared under similar conditions, one such batch being alkali refined linseed oil, without any modifying agent, and the other being alkali refined linseed oil containing 2% resorcinol alone (without the sulpho-salicylic acid).

All three of the above oils were then heat bodied to a viscosity of from Z-4 to Z-6 and 25 gallon long ester gum varnishes were prepared with the bodied oils in the manner described above, the several varnishes being tested in the manner described above, and giving the following results:

Table No. V

| Ex. No.        | Modifying agent               | Minutes cooking of varnish | Viscosity of varnish | Drying         | Hot water | Cold water | Alkali                             |
|----------------|-------------------------------|----------------------------|----------------------|----------------|-----------|------------|------------------------------------|
| 18             | 2% resorcinol + 5% sulpho-sal | 172                        | E                    | Fair           | Very good | Very good  | Good after 7 hrs.; gone overnight. |
| D <sub>v</sub> | Oil without any agent         | 135                        | E                    | Fair +<br>Good | Good      | Good       | Gone 2 hrs.                        |
| E <sub>v</sub> | 2% resorcinol                 | 116                        | C                    | do             | Fair      | Fair       | Gone 3½ hrs.                       |

Although the above table indicates that the sulpho-salicylic acid slightly decreases the bodying speed and the drying velocity of the resorcinol treated oil, it is noted that the presence of the sulpho-salicylic acid contributes to very good hot and cold water resistance and also greatly increases the alkali resistance. (It may be mentioned that for the alkali tests in Table V films of only .0015 inch thickness were employed, which is in contrast to the heavier films (.0030) used in other examples.)

## EXAMPLE 19

A batch of 1,200 gms. of alkali refined linseed oil was refluxed with 2% resorcinol at 150° C. Thereafter, 0.5% of naphthionic acid was added to the oil and the temperature raised to 300° C. for 5½ hours, under a blanket of CO<sub>2</sub>. This secured a viscosity of Z-5 and from this treated oil a 25 gallon long ester gum varnish was prepared in accordance with the above description, yielding after a 2½ hour cooking at 300° C., a viscosity of D, at 50% solids. The resulting varnish had substantially improved alkali resistance compared to that of a similar varnish made with a similar oil containing resorcinol alone. The drying velocity, cold water and boiling water resistance were somewhat better than that of the varnish made with an oil treated only with resorcinol.

## EXAMPLE 20

A batch of 4000 gms. of alkali refined linseed oil were treated with 5% maleic anhydride and 2% resorcinol, by refluxing the reaction mixture for two hours at 150° C. After the precondensation period, the reflux condenser was eliminated and the temperature of the oil raised to 295° C. for 2 hours and 10 minutes, yielding a viscosity of V.

Here again a 25 gallon long ester gum varnish

was prepared in the manner already described, yielding in the short time of 60 minutes a viscosity of G at 50% solids (cut with mineral spirits).

Although the alkali resistance of the varnish was somewhat reduced as compared with a varnish containing an oil made with resorcinol alone, by the conjoint use of maleic anhydride the bodying velocity was greatly increased, and in addition, the drying time, cold water and boiling water resistance, were all very satisfactory.

## EXAMPLE 21

In this example, a compound treatment of still another type is illustrated. For this purpose a treated linseed oil was employed as a starting material, the oil containing beta-methyl-anthraquinone as an agent for accelerating heat bodying. This oil had a viscosity about the same as alkali refined or raw linseed oil.

Seventy pounds of the treated oil were heated in a 15 gallon kettle with 2% resorcinol under reflux for 2 hours at 150° C. A 5,000 gm. batch of the resorcinol treated oil was then bodied at

300° C. for two hours and twenty minutes, under a blanket of CO<sub>2</sub>, yielding a viscosity of X.

The foregoing treated and heat bodied oil was then employed in the preparation of 25 gallon long varnishes prepared in the general manner described above. Three such varnishes were prepared using different resins, as follows:

- Ester gum.
- Paranol 1750 (a rosin modified phenolic resin).
- Amberol 801 (a rosin modified maleic resin).

The three varnishes were then cooked to a viscosity of C to H, at 50% solids when diluted with mineral spirits and when containing the drier combination hereinabove described. The bodying times and viscosities are indicated in the following table.

Table VI

| Ex. No. | Resin        | Minutes cooking | Viscosity |
|---------|--------------|-----------------|-----------|
| 21a     | Ester gum    | 315             | K         |
| 21b     | Paranol 1750 | 35              | C         |
| 21c     | Amberol 801  | 65              | I         |

The foregoing varnishes were subjected to tests of the types described above, the results indicating that the cold water and boiling water resistance were somewhat improved as compared to a similar varnish made with oil containing beta-methyl-anthraquinone, but not containing resorcinol. The drying properties and alkali resistance were both substantially improved as compared with the varnishes not containing resorcinol.

The most striking improvement, however, is the increase in the rate of bodying, as compared with linseed oil treated with resorcinol alone.

For purposes of comparison between varnishes (or varnish bases) prepared with the oil treated only with beta-methyl-anthraquinone, and with

13

said oil further treated with resorcinol, it may be noted that, if properly pre-bodied to a viscous oil, it will be found that in the cooking of varnishes (or varnish bases) the oil (without resorcinol) will further body fairly rapidly. The addition of resorcinol to the treated oil (containing beta-methyl-anthraquinone) imparts a slight but still further increase in bodying velocity. Such acceleration of bodying is noticeable, for instance with varnishes (or varnish bases) prepared with ester gum. However, the more important improvement imparted to this treated oil by the further addition of resorcinol is the improvement in drying and also some of the other properties, for instance alkali resistance.

It, therefore, appears that such conjoint treatment with resorcinol and certain other agents not only achieves the advantages of resorcinol, but at the same time secures other improvements in properties, notably the velocity of bodying.

Particularly useful products may be secured by conjoint treatment with a polyhydroxy benzene and with other modifying agents such as organic acids (polycarboxylic acids), condensed ring compounds and organic sulfonic acids, examples of which are given in my Patents 2,298,914, 2,298,915 and 2,298,917.

In four examples referred to below, oils were treated in accordance with this invention, with somewhat different procedures in each case. Thereafter, comparative varnish formulas were made employing these oils. The treatment of the oils is first referred to just below under individual example numbers, following which the varnish preparation and results are described.

#### EXAMPLE 22

A batch of 150 gms. of linseed oil was heated in a 500 cc. Erlenmeyer flask with 7½ gms. of resorcinol for 5 hours at a temperature between about 200 and 220° C., the batch being kept under a vacuum of 26 to 29 inches. The temperature was just below the boiling point and the treated oil was a somewhat bodied clear mobile oil. Although no extensive changes were visible in the oil itself, improved properties were secured in varnishes, as brought out below.

#### EXAMPLE 23

A batch of 150 gms. of linseed oil was heated in an open beaker with 7½ gms. of resorcinol for 3 hours at a temperature from 180° C. to 200° C., for the purpose of precondensation. Thereafter the temperature was raised to 285° C. and the product kept at or somewhat above that temperature for 5 hours. In the final half of the bodying period, the temperature was between 300 and 320° C. After about 2½ hours of the heat bodying, the oil started to body very rapidly.

#### EXAMPLE 24

A batch of 150 gms. of linseed oil was heated with 15 gms. of resorcinol in a Pyrex flask under air reflux. Solution of the resorcinol had been attained when the temperature rose to 220° C. yielding an amber colored oil. At about 306° C. the batch was simmering gently, but developed some vigorous bumping, so that for a short time the refluxing was replaced by a distillation connection. Very little of the material distilled. The refluxing was continued at 300° C. until, after 1½ hours, the reflux condenser was taken off, heating being continued under open atmospheric conditions at 280° C. to 300° C. for 3½ hours. The total time between 280° and 306° C. was 6 75

14

hours, and the product at this stage was a fairly thin clear oil.

The treated oil was thereafter further heated by continuing heating at 290° to 310° C. for two hours, after which heating the oil was considerably thicker. After cooling overnight, the batch was again heated for a further period of 2½ hours at the same temperature (290° to 310° C.), and during this time the oil became gradually thicker. Finally the oil was of a semi-solid consistency when cooled to room temperature.

#### EXAMPLE 25

A batch of linseed oil was heated in a manner similar to that described above in connection with Example 23, the treating agent, however, being Pyrogallol (1, 2, 3, trihydroxy benzene) instead of resorcinol. The oil was heated between 170 and 200° C. for 3 hours and then between 20: 280 and 300° C. for 4 hours, and finally kept at 320° C. for 50 minutes. No appreciable bodying took place until the temperature exceeded about 300° C., but thereafter the bodying was rapid and the final product, when cold, was a gelatinous solid.

#### COMPARATIVE EXAMPLES 22v TO 25v

The final oil products of Examples 22 to 25 were employed in the preparation of batches of varnishes made of 25 gallon length with lime hardened rosin, the varnishes being diluted to 50% solids with mineral spirits. These varnishes were tested for drying and other properties and in each case, the varnish was tested in four different forms as follows:

- a. Varnish without drier.
- b. Varnish plus cobalt drier (0.03 cobalt metal on the basis of oil content).
- c. Zinc oxide paint made with the varnish without drier (pigment to vehicle solids ratio=1 to 1 by weight).
- d. Zinc oxide paint as per c, with drier as per b.

For comparative purposes, a blank series of varnishes and paints were also made up from a medium bodied linseed oil not containing any modifying agent.

In the drying tests one of the most significant results which showed up was the considerable improvement in all of the varnishes made with treated oils as compared with the blanks, with respect to "after-tack." The varnishes made with the treated oils were very much more "print-free" than is usual with soft oil varnishes.

In the varnishes not containing cobalt drier, the rate of drying of the varnishes containing the treated oils was also improved as compared with the blanks, the several examples showing up in the following order, the best drying being placed at the top of the list and being far superior to the following:

- Varnish made with oil of Example 24, containing 10% resorcinol.
- Varnish made with oil of Example 23, containing 5% resorcinol.
- Varnish made with oil of Example 25, containing 5% Pyrogallol.
- Varnish made with oil of Example 22, containing 5% resorcinol.

In the varnishes containing cobalt drier, the drying results were also quite satisfactory, the varnishes made with oils of Examples 23 and 22 (both containing 5% resorcinol) being the best.

In the paints not containing cobalt drier the results were similar to the varnishes, the four examples maintaining the same order as above noted, and at least the first three (in that order being improved as compared with the blank and the four being about equal to the blank).

In the paints containing cobalt drier, the biggest improvement was indicated in the initial drying, the best result in this regard being secured with the paint made with the treated oil of Example 25 (containing 5% pyrogallol).

Another significant improvement which showed up in the tests of the foregoing varnishes and paints was that notwithstanding the use of lime hardened rosin as the resin ingredient, very good water resistance was secured, especially in the paints made with the oils of Examples 25, 23 and 24, and with the clear varnish made with the treated oil of Example 25.

I claim:

1. A process for treating fatty oils having drying properties to improve their characteristics, as components of surface coating compositions, which process comprises incorporating in the oil up to 30% of resorcinol as the sole active treating agent, and heating the mixture at a temperature between the dissolution point of the resorcinol and about 310° C. for at least 30 minutes.

2. A process in accordance with claim 1 in which the heating of the oil containing resorcinol is effected in two stages, the first of which is continued for at least 30 minutes at a temperature not exceeding about 200° C. and the second of which is continued for at least 30 minutes at a temperature above about 200° C.

3. A process in accordance with claim 1 in which the heating of the oil containing resorcinol is effected in two stages, the first of which is continued for at least 30 minutes at a temperature not exceeding about 200° C. and the second of which is continued for at least 30 minutes at a temperature above about 200° C., said first stage being carried out under refluxing conditions.

4. A process for treating fatty oils having drying properties, to improve their characteristics as components of surface coating compositions, which process comprises incorporating in the oil up to 10% of resorcinol as the sole active treating agent, and heating the mixture under refluxing conditions at a temperature between about 75° C. and about 250° C. for at least 30 minutes.

5. A process in accordance with claim 4 and further comprising additionally heating the refluxed mixture at a temperature between about 250° C. and about 310° C. for at least 30 minutes.

6. A process for treating fatty oils having drying properties, to improve their film-forming characteristics when used as components of surface coating materials, which process comprises incorporating in the oil up to 30% of a polyhydroxy benzene as the sole active treating agent, and heating the mixture at a temperature between about 75° C. and about 350° C. but not above the boiling or decomposition point of the oil, whichever is lower, for at least 30 minutes.

7. A process for treating fatty oils having drying properties, to improve their film-forming characteristics when used as components of sur-

face coating materials, which process comprises incorporating in the oil up to 30% of a polyhydroxy benzene as the sole active treating agent, and heating the mixture at a temperature between about 75° C. and about 310° C. for at least 30 minutes.

8. A process in accordance with claim 7 in which said polyhydroxy benzene is a dihydroxy benzene.

9. A process in accordance with claim 7 in which said polyhydroxy benzene is a trihydroxy benzene.

10. A process in accordance with claim 7 in which said polyhydroxy benzene is pyrogallol.

11. A process for treating fatty oils having drying properties, to improve their film-forming characteristics when used as varnish base materials, which process comprises incorporating in the oil up to 10% of resorcinol as the sole active treating agent, and heating the mixture at a temperature between about 75° C. and about 310° C. for at least 30 minutes.

12. A process in accordance with claim 11 in which at least a portion of the heating is effected under refluxing conditions.

13. A process in accordance with claim 11 in which an initial portion of the heating is effected at a relatively low temperature under refluxing conditions, and in which a succeeding portion of the heating is effected at a relatively higher temperature sufficient to effect heat bodying.

14. A process in accordance with claim 11 in which the fatty oil is selected from the class comprising drying fatty oils and semi-drying fatty oils.

15. A process in accordance with claim 11 in which the fatty oil is linseed oil.

16. A process in accordance with claim 11 in which the fatty oil is soya bean oil.

17. A process in accordance with claim 11 in which the fatty oil is a pentaerythritol ester containing linseed oil fatty acids.

18. A varnish comprising a fatty oil containing from about .05% to about 30% of resorcinol as the sole added treating agent, a varnish resin and a volatile solvent.

19. A varnish comprising a fatty oil containing from about .05% to about 30% of pyrogallol as the sole added treating agent, a varnish resin and a volatile solvent.

20. A process for treating fatty oils having drying properties to improve their film-forming characteristics when used as components of surface coating compositions which process comprises incorporating in the fatty oil up to 5% of resorcinol as the sole active treating agent, precondensing the resorcinol with the oil at a temperature below about 250° C. and thereafter heat bodying the oil by heating the mixture to a heat bodying temperature above about 250° C.

21. A process in accordance with claim 4, in which the quantity of resorcinol used is between 1/2% and 2% of the weight of the oil.

22. A process in accordance with claim 11, in which at least a portion of the heating is effected under refluxing conditions and the temperature of the refluxing being at least 150° C. and not more than 200° C. and the refluxing time being at least 30 minutes.

70 LASZLO AUER.